

# UNITED STATES PATENT OFFICE.

WILSON H. STRICKLER, OF DODGE CITY, KANSAS.

## LUBRICANT.

SPECIFICATION forming part of Letters Patent No. 476,574, dated June 7, 1892.

Application filed April 6, 1891. Serial No. 387,723. (No specimens.)

*To all whom it may concern:*

Be it known that I, WILSON H. STRICKLER, a citizen of the United States, residing at Dodge City, in the county of Ford and State 5 of Kansas, have invented a new and useful Improvement in Lubricants and Steam-Pack-  
ing for Steam-Engines, Journals, Bearings, Steam-Chests, Boilers, Steam and Hot-Air  
Pipes, and in general such parts of machinery  
10 as are exposed to friction or the effects of heat;  
and I do hereby declare the following to be a full, clear, and exact description of the invention,  
such as will enable others skilled in the art to which it appertains to make and use  
15 the same.

My invention consists in the application of the minerals asbestos, soapstone, and mica in combination to the purpose of a lubricant and packing for machinery, and the mode in which  
20 I prefer to practice my invention is as follows:

The asbestos, soapstone, and mica are pul-  
verized in a mill or by any other suitable  
means, and in this pulverized condition, prefer-  
ably in about equal quantities, (more or  
25 less,) are mixed with oil and applied to the  
part to be lubricated. The pulverized asbes-  
tos, while overcoming the effects of heat and  
friction, also holds the pulverized soapstone  
and mica in suspension in the oil, thereby ma-  
30 terially bettering its form and quality as a  
lubricant, and, being fibrous and expansive,  
makes a tight and most effective packing. The  
laminated surfaces of the mica take up and

hold in contact the oil, as well as the pulver-  
ized asbestos and soapstone. No matter how 35  
finely pulverized, the mica possesses a large  
surface of contact for the adhesion of these  
substances. Soapstone is not a necessary in-  
gredient of my composition; but I prefer ordi- 4c  
narily to use it, as it imparts a desirable qual-  
ity to the lubricant. When used as a steam-  
packing for engines, boilers, steam and hot-  
air pipes, &c., it is mixed with cotton or any  
suitable fibrous material. In this manner it  
is used as a packing or sheathing for all parts 45  
of machinery conveying steam or heat.

I am aware that mica, soapstone, oil, and  
asbestos have heretofore been used separately  
and in combinations as lubricants, and I there-  
fore lay no claim to the use of these sub- 50  
stances or any of them separately, but only  
to the particular combinations hereinafter  
claimed, which I am not aware have hereto-  
fore been used or patented and which I have  
discovered possess peculiar advantages. 55

What I claim as my invention, and desire to  
secure by Letters Patent of the United States,  
is—

A composition of pulverized asbestos, soap-  
stone, mica, and oil, substantially as described. 60

In testimony whereof I affix my signature in  
presence of two witnesses.

WILSON H. STRICKLER.

Witnesses:

A. N. BOOREY,  
L. E. McGARRY.